

E. M. CHADBOURNE.  
ASPHALTIC PAVEMENT.  
APPLICATION FILED JAN. 7, 1914.

1,103,127.

Patented July 14, 1914.

Fig. 1.



Fig. 2.



Fig. 3.



Fig. 4.



Inventor

Witnesses

Harley R. Brown,  
M. P. Crandall

By

E. M. Chadbourne  
Church & Church  
his Attorneys

# UNITED STATES PATENT OFFICE.

EDWARD M. CHADBOURNE, OF TACOMA, WASHINGTON.

## ASPHALTIC PAVEMENT.

1,103,127.

Specification of Letters Patent.

Patented July 14, 1914.

Application filed January 7, 1914. Serial No. 810,866.

*To all whom it may concern:*

Be it known that I, EDWARD M. CHADBOURNE, a citizen of the United States, residing at Tacoma, in the county of Pierce and State of Washington, have invented certain new and useful Improvements in Asphaltic Pavements; and I do hereby declare the following to be a full, clear, and exact description of the same, reference being had to the accompanying drawings, forming part of this specification, and to the figures and letters of reference marked thereon.

This invention relates to the construction of pavements for roadways and more especially to that type wherein the surface is formed by a rock or stone aggregate combined with an asphaltic binder which is substantially non-fluid at ordinary temperatures, but is capable of being rendered limpid or liquid by the application of heat. The surface layer is usually supported by a suitable foundation such as cement or concrete and approved practice indicates the desirability of forming the surface of the foundation with pockets or irregularities, for example, such as referred to in my prior Patent No. 994,092.

The present invention is designed particularly as an improvement upon the process of my said prior patent, the objects being to simplify the process of laying the pavement to make a more uniform and homogeneous aggregate, reduce the temperature necessarily employed, and to do away as far as possible with the necessity of handling any of the ingredients in a mixed condition, thus avoiding the necessity of long hauls and expensive mechanical mixing plants.

As in my said prior patented process, the present process contemplates also the use of an agglomerate which in its final condition is substantially free from voids and is thoroughly bonded together with no excess of either asphalt binder or aggregate. To accomplish this result and secure the thorough distribution of the asphaltic binder, and its retention in the aggregate by surface tension, thus overcoming any tendency to drain away, the aggregate must be of such proportions as to have from twenty-five to forty per cent. of voids, for it is within these limits that effective capillary action will take place and the binder be held against draining away or accumulating in excess at low spots.

Considerable difficulty is experienced in obtaining an asphaltic binder which is uniformly sufficiently limpid when heated, to accomplish the desired result of distribution through the heated aggregate entirely by capillary action. The difficulty is due to the fact that many asphaltic binders are treated with dust, lime, etc., to give them body, and most of the natural asphalt binders, such as the Bermudez or Trinidad asphalts naturally contain a large amount of sediment, and this dust, lime or sediment, no matter whether purposely placed in the asphalt, or found naturally therein, has a tendency to clog up the passages through which the asphalt should feed by capillary action, and with the result that a uniform distribution of the binder is interfered with. So, also, where capillary attraction alone is relied upon, the aggregate must be heated to a very high temperature in order to maintain the asphalt in a limpid condition for a sufficient length of time to effect the uniform distribution. Besides adding to the cost, the heating of the aggregate to a very high temperature always involves the risk of burning the asphalt or causing its quality to deteriorate, and the resultant mixture may contain a larger percentage of binder than is necessary to secure the best results, for it is obvious that where the binder is not uniformly and evenly distributed, but is in excess at some points, the pavement will be unnecessarily soft in hot weather where such excess exists, and this may result in its destruction under heavy traffic conditions.

The present invention is designed to overcome many, if not all, of these defects which could not be foreseen but have been, to a considerable extent, developed in the practical work of laying pavements.

In carrying the invention into effect, the heated aggregate and binder are separately placed in layers of proper thickness on the previously prepared base, the aggregate being in a heated condition, but the temperature need not be so high as that found to be necessary where the materials remain without being disturbed after their disposition, for, in the present instance, after the materials are distributed in layers they are mechanically mixed *in situ* by being turned over and over so that the capillary action which takes place may proceed from various points of distribution, so to speak, inasmuch as the asphalt binder will be stirred up into the

aggregate. The mechanical mixing of the aggregate and binder *in situ* is preferably effected by drawing a rake-like implement backward and forward through the same, so as to effect a thorough stirring without causing the materials to segregate by reason of their difference in weight or size. Inasmuch as the binder is mechanically distributed through the aggregate it is obvious that the heat required is considerably less, as is also the time necessary to be allowed for the complete distribution of the binder by capillary action.

In practice it is preferred to first spread the asphalt binder with a suitable templet, to the desired depth, said binder being of the character referred to which is not limpid or liquid at ordinary temperatures. The depth of the layer of asphalt binder varies in accordance with the particular character of aggregate, and it is preferably determined empirically in a known way. Having spread the asphalt binder, the heated aggregate is next spread, with a templet so as to secure a proper proportion of the same, over the layer of binder and this aggregate is composed of broken rock, sand and dust, or of sand and dust alone, depending upon whether sheet asphalt or an asphaltic concrete pavement is desired. The use of templets is very essential for, by means of them the depth of any layer or the proportion of asphalt and aggregate may be accurately determined with great uniformity. As soon as the hot aggregate has melted the asphalt binder the raking and stirring is commenced, and is continued until a thorough uniform mixture will result by a comparatively quick and uniform capillary action. After this stirring operation, the pavement is rolled in the well understood manner, and in accordance with common practice.

Referring to the accompanying drawings, Figure 1 is a sectional view through a base with an asphalt binder spread evenly over the same; Fig. 2 shows the binder covered by an aggregate of hot sand and rock, the latter having been spread with templets to the desired depth. Fig. 3 illustrates a rake with vaned prongs, arranged to mechanically mix and combine the asphalt and aggregate when drawn and pushed back and forth through the same; and Fig. 4 is a view showing the pavement completed and rolled.

In said drawings, the letter A indicates the base; C, the layer of normally non-fluid asphaltic binder spread on the base to a uniform depth.

D is the hot layer of aggregate preferably having between twenty-five and forty per cent. of voids.

F is the rake having the vaned prongs *f* for mixing the aggregate and binder after the binder has been rendered more or less 65 limpid by the heat of the aggregate, and G indicates the finished pavement in which the aggregate and binder have been distributed to form a homogeneous mass, and the mass has been rolled or condensed by surface pressure in the ordinary way.

Having thus described my invention, what I claim as new and desire to secure by Letters Patent of the United States, is:

1. The method of constructing pavements 75 composed of aggregate bonded together by an asphaltic binder which is non fluid at ordinary temperatures but capable of being rendered limpid by the application of heat, which consists in distributing the asphaltic binder and aggregate separately on a prepared foundation in layers of the proper depth to give the desired proportions when the layers are commingled, and in reducing the binder to a limpid condition 80 by heating the same, then stirring the aggregate and binder *in situ* on the prepared foundation, and finally condensing the commingled aggregate and binder by surface pressure. 90

2. The method of constructing pavements composed of aggregate having its voids filled and the particles bonded together by asphaltic binder, which consists in spreading a layer of asphaltic binder on a suitable 95 base, then spreading a loose layer of heated aggregate over the same, the thickness of the two layers being such as to give the proper proportions for the pavement when mixed, then mixing the layers of binder and 100 heated aggregate by stirring the same on the base, then compacting the mixed aggregate and binder by surface pressure.

3. The method of constructing pavements, having a layer of mingled aggregate with 105 its voids filled and the particles bonded together by asphaltic binder non-fluid at ordinary temperatures but capable of being rendered limpid by heat, which consists in spreading separately a layer of asphaltic 110 binder, and a layer of heated aggregate having between twenty-five and forty per cent. of voids therein, one over the other on a suitable roadway foundation, and in stirring the two layers together, whereby 115 capillary action is hastened by the mechanical distribution of the binder through the layer of aggregate and uniform distribution of the binder is insured, and finally compacting the same by surface pressure. 120

EDWARD M. CHADBOURNE.

Witnesses:

J. W. STOUT,  
A. SKOYEN.